

## 1

2,727,841

## METHOD AND COMPOSITION FOR IMPROVING CORROSION RESISTANCE OF ZINC

Allan E. Chester, Highland Park, Ill., assignor to Poor &amp; Company, Chicago, Ill., a corporation of Delaware

No Drawing. Application November 30, 1950,  
Serial No. 198,490

9 Claims. (Cl. 148—6.2)

This invention relates to a method of improving the corrosion resistance of zinc surfaces and to a one-step process for effecting such improvement.

It is well known that zinc surfaces tend to turn white or grayish white with age, a property sometimes referred to as "white corrosion," which is apparently due to the formation of oxides and carbonates. Several processes have been devised for increasing the resistance of zinc surfaces to "white corrosion." One of these involves dipping the article made of zinc or containing a zinc coating in a chromic acid bath. The resultant product, however, discolors and therefore leaves much to be desired.

Another method of treating zinc surfaces is the so-called "bright dip" wherein the zinc article or an article containing a zinc coating is dipped in a bath of chromic acid anhydride, sodium sulfate and nitric acid. This process has the disadvantage that the articles are hard to rinse and the bath has no substantial passivating effect on the zinc.

Improved brightness in articles containing an electroplated coating of zinc has been obtained by adding various types of addition agents to the electroplating bath. This process is also used in conjunction with a "bright dip" of the type previously described.

Several processes have been described in the literature which are said to produce a bright zinc plate. One of these involves the treatment of a zinc plated article with a chromic acid bath containing a sulfate radical in a critical ratio followed by treatment in a second step with a solution of an acid having a pH less than 2.68. Another process involves a treatment in one step with a chromic acid bath and in a second step with a caustic alkali solution having a normality between 4.25 and saturation. Still a third process involves a treatment in which glacial acetic acid is employed with chromic acid in a first bath followed by a caustic dip in the second bath.

It will be observed that in many of the previously described processes the zinc surfaced article must be given a primary treatment and a secondary treatment.

One of the objects of the present invention is to provide a new and improved method of treating zinc articles or articles containing a surface coating of zinc to produce zinc surfaces which are resistant to white corrosion.

A further object is to provide a method of the character described which requires treatment of the zinc article or zinc surfaced article in a single bath only, followed by rinsing.

An additional object is to provide new and useful compositions for protecting zinc.

Another object of the invention is to provide a chromic acid bath for treating zinc or zinc surfaced articles which does not produce the brown discoloration normally characteristic of such baths. Other objects will appear hereinafter.

In accomplishing these objects in accordance with this

## 2

invention it has been found that new and improved results in producing zinc coatings of enhanced corrosion resistance can be obtained by subjecting zinc or a zinc coated article to treatment with a nitric acid bath containing chromic acid and a fluorine compound.

The products produced in accordance with the invention will withstand 24 to 100 hours salt spray before the appearance of white corrosion as against two hours for unprotected zinc. A higher degree of protection has been obtained by more elaborate and expensive methods but the present invention provides an inexpensive single step treatment and the products are satisfactory for many uses where greater protection is not required.

It is believed that the improved results obtained in the practice of the invention are due to the fact that the fluorine apparently whitens and brightens zinc and permits the chromic acid and nitric acid to attack the zinc surface uniformly. Also, it is believed that as zinc goes into solution the pH at the interface between the zinc surface and the solution changes rapidly. In some unexplained manner fluorine compounds, as, for example, trifluoroacetic acid and fluoboric acid in the presence of nitric acid prevent the formation of brown chromium chromates and permit chromium oxides to form. Thus, the invention eliminates the necessity for a secondary operation to remove the brown chromium chromates which normally stain zinc surfaces that have been treated in chromic acid bath. The treated zinc coatings produced in accordance with the invention are very receptive to paints and paint enamels whereas ordinary zinc surfaces cannot be painted satisfactorily.

The invention contemplates the preparation of the chromic acid and fluorine compounds, with or without auxiliary agents, as addition agents for nitric acid treating baths. The brightness of the resultant treated surface can be increased by increasing the concentration of the nitric acid. For example, the compositions of the invention may be added to a nitric acid bath containing 0.5 to 5% HNO<sub>3</sub>. Where brightness is not particularly desired, the concentration of HNO<sub>3</sub> may be relatively low, for example, 0.5 to 1.5% by weight. On the other hand, if brightness is desired it can be obtained by employing 2% to 5% by weight of HNO<sub>3</sub>.

The invention will be illustrated but is not limited by the following example.

*Example*

A composition was prepared by mixing together the following ingredients:

380 lbs. magnesium sulfate  
190 lbs. sodium dichromate  
47.5 lbs. chromic acid  
864 cc. trifluoroacetic acid

This mixture was added to 200 gallons of water and agitated in a lead-lined tank. Additional water was added sufficient to make 396 gallons. The resultant composition was then added to carboys in the proportion of 99.5 lbs. for each carboy and to each carboy was also added 11.5 lbs. of fluoboric acid. The carboys were then capped and stored.

If a stainless steel tank is used in mixing, the fluoboric acid can be added with the other ingredients, a total of 412.5 lbs. being required.

The chromic acid content of the concentrate in this example is approximately 1.82 grams per gallon. The fluorine compounds content is approximately 1.59 grams per gallon, calculated as fluorine (F).

In the previously described composition the magnesium sulfate is employed to inhibit the attack of nitric acid on the zinc surface when the composition is employed

as an addition agent to a nitric acid bath as hereinafter described.

The foregoing concentrate composition is employed as an addition agent to a nitric acid bath consisting of 0.5 to 5% HNO<sub>3</sub> by weight dissolved in water in proportions from 1:19 to 1:99 by weight, preferably 1 part of concentrate to 49 parts of dilute HNO<sub>3</sub>.

The quantity of the addition agent employed may vary but is preferably such that the concentration of chromic acid (CrO<sub>3</sub>) in the bath is within the range of about 1.82 grams per gallon to 9.1 grams per gallon of bath. It will be understood that the dichromate originally present in the addition agent is also considered in calculating the chromic acid content of the bath.

It will be understood that the fluoboric acid may be replaced entirely by trifluoroacetic acid on an equivalent fluorine basis. It is also possible to use all fluoboric acid. The fluorine content of the addition agent may range from about 1.59 to 7.95 grams per gallon of solution and it may be replaced wholly or in part by inorganic fluorine compounds, as, for example, sodium acid fluoride or sodium fluoride. Esters of fluoboric acid and trifluoroacetic acid can be used instead of the free acids, for example, the methyl, ethyl, propyl and butyl esters as well as their higher homologues.

The relative proportions of the various ingredients given in the example are those which will produce approximately optimum results. The chromic acid and fluorine contents of the treating bath are preferably approximately 3.64 and 3.18 grams per gallon, respectively.

Because it contains a greater concentration of fluorine all trifluoroacetic acid is preferably employed rather than a mixture of trifluoroacetic acid and fluoboric acid. However, in the commercial formula illustrated in the example fluoboric acid is used because it provides a cheaper source of fluorine. It is generally less desirable to use fluorides because of their lower solubility in the bath and the formation of hydrogen fluoride. Hydrogen fluoride can be used as such but suffers from the disadvantage that it attacks glass and therefore compositions containing it would require special types of containers. As will be apparent, the fluorine containing acid forms only a fraction of a per cent by weight of the treating bath.

In the practice of the invention the zinc surfaced article is merely dipped in the nitric acid bath containing the aforesaid addition agent and then rinsed. As an illustration, zinc is plated onto steel in a conventional bath without adding any brightening agents. A typical conventional zinc plating bath has the following composition:

95-100 grams sodium cyanide  
45-55 grams zinc metal (added as the chemically equivalent proportion of zinc oxide)  
100-120 grams sodium hydroxide and enough water to make 1 liter of solution

2 grams per liter of zinc dust are stirred into the electrolyte, and the entire mixture is filtered in order to remove traces of heavy metals.

The plated article is then rinsed and dried or without drying is immersed in a bath made by adding the previously described addition agent to a solution of 0.5 to 5% by weight HNO<sub>3</sub>. The bath is preferably at room temperature (75 degrees F.) and the article is immersed in the bath from 1 to 15 seconds. Thereafter it is removed and thoroughly rinsed with water. It will be found that the corrosion resistance of the zinc coating has been increased and an article having an excellent appearance is obtained. As previously indicated, if it is desired to produce a very bright zinc plate the quantity of nitric acid should preferably be at least 2% by weight of the bath.

The invention makes it possible to provide a zinc surface which is resistant to white corrosion and if desired

to produce a very bright zinc surface. This is accomplished by a simple one-step treatment which avoids the formation of brown, water soluble chromium chromate salts, eliminates the necessity for secondary operations to remove discoloring brown stains caused by such salts and at the same time provides a very uniform coating of enhanced brightness. The quantities of CrO<sub>3</sub> required are relatively low. The coatings produced on zinc by the present invention not only are pleasing to the eye when allowed to remain as such, but also are receptive to paint and enamels and can be painted or enameled without the usual chipping or peeling that occurs when untreated zinc surfaces are painted or enameled.

It will be understood that the word "enamel" as used herein refers to paint enamels rather than vitreous enamels.

The expression "zinc surfaced article" is employed herein to cover any article having an exterior surface of zinc regardless of whether the article is made entirely of zinc or whether it has a zinc coating. The expression "zinc plated article" is employed herein to describe a zinc coated article in which the zinc coating has been applied by an electroplating process.

The invention is hereby claimed as follows:

1. A process of protecting zinc against corrosion which comprises treating a zinc surfaced article with an aqueous solution consisting essentially of 0.5 to 5% by weight HNO<sub>3</sub>, 1.82 to 9.1 grams per gallon of CrO<sub>3</sub> and 1.59 to 7.95 grams per gallon of fluorine in the form of a water soluble fluorine-containing compound from the group consisting of trifluoroacetic acid, fluoboric acid and the lower alkyl esters of said acids.

2. A composition for treating zinc surfaces in order to protect the zinc against corrosion, said composition consisting essentially of an aqueous solution of chromic acid, nitric acid, fluoboric acid and trifluoroacetic acid, the quantity of chromic acid being within the range of 1.82 to 9.1 grams per gallon, the quantity of nitric acid corresponding to 0.5 to 5% by weight, and the quantity of said fluorine-containing acids calculated as fluorine being within the range from 1.59 to 7.95 grams per gallon.

3. An addition agent adapted to be added to a nitric acid solution to provide a bath for protecting zinc surfaces against corrosion consisting essentially of approximately 380 lbs. magnesium sulfate, approximately 190 lbs. sodium dichromate, approximately 47.5 lbs. chromic acid, and approximately 864 cc. trifluoroacetic acid dissolved in sufficient water to make approximately 396 gallons and approximately 412.5 lbs. fluoboric acid.

4. A process of protecting zinc against corrosion which comprises treating a zinc surfaced article with an aqueous solution consisting essentially of 0.5 to 5% by weight HNO<sub>3</sub>, 1.82 to 9.1 grams per gallon of CrO<sub>3</sub> and 1.59 to 7.95 grams per gallon of fluorine in the form of fluoboric acid.

5. A process of protecting zinc against corrosion which comprises treating a zinc surfaced article with an aqueous solution consisting essentially of 0.5 to 5% by weight HNO<sub>3</sub>, 1.82 to 9.1 grams per gallon of CrO<sub>3</sub> and 1.59 to 7.95 grams per gallon of fluorine in the form of trifluoroacetic acid.

6. A process of protecting zinc against corrosion which comprises treating a zinc surfaced article with an aqueous solution consisting essentially of 0.5 to 5% by weight HNO<sub>3</sub>, 1.82 to 9.1 grams per gallon of CrO<sub>3</sub> and 1.59 to 7.95 grams per gallon of fluorine in the form of fluoboric acid and trifluoroacetic acid.

7. A composition for treating zinc surfaces consisting essentially of an aqueous solution of 0.5 to 5% by weight HNO<sub>3</sub>, 1.82 to 9.1 grams per gallon of CrO<sub>3</sub> and 1.59 to 7.95 grams per gallon of fluorine in the form of a water soluble fluorine-containing compound from the group consisting of trifluoroacetic acid, fluoboric acid and the lower alkyl esters of said acids.

8. A composition for treating zinc surfaces in order to

protect the zinc against corrosion, said composition consisting essentially of an aqueous solution of 1.82 to 9.1 grams per gallon of  $\text{CrO}_3$ , 0.5 to 5% by weight of  $\text{HNO}_3$  and 1.59 to 7.95 grams per gallon of fluorine in the form of trifluoroacetic acid, the relative proportions of said ingredients being sufficient to enhance the corrosion resistance of zinc while avoiding the formation of brown stains on the zinc surface when said composition is applied thereto.

9. An addition agent adapted to be added to a nitric acid solution to provide a bath for protecting zinc surfaces against corrosion consisting essentially of a chromium compound which forms chromic acid in the presence of an acid and a fluorine-containing compound from the group consisting of trifluoroacetic acid, fluoboric acid and the lower alkyl esters of said acids, the proportions of said substances in said addition agent being such that said addition agent can be dissolved in water to produce a solution containing 1.82 to 9.1 grams per gallon of

$\text{CrO}_3$  and 1.59 to 7.95 grams per gallon, calculated as fluorine, of said fluorine-containing compound.

References Cited in the file of this patent

UNITED STATES PATENTS

|           |                      |                |
|-----------|----------------------|----------------|
| 2,288,007 | Lum                  | June 30, 1942  |
| 2,296,884 | Thompson             | Sept. 29, 1942 |
| 2,376,158 | McCarroll et al.     | May 15, 1945   |
| 2,428,749 | De Long              | Oct. 7, 1947   |
| 2,471,909 | Spruance, Jr.        | May 31, 1949   |
| 2,483,510 | Stareck              | Oct. 4, 1949   |
| 2,494,909 | Spruance, Jr. et al. | Jan. 17, 1950  |
| 2,524,577 | Stareck              | Oct. 3, 1950   |
| 2,593,447 | Hesch                | Apr. 22, 1952  |
| 2,593,448 | Hesch                | Apr. 22, 1952  |
| 2,613,165 | Fischer              | Oct. 7, 1952   |

FOREIGN PATENTS

|         |             |              |
|---------|-------------|--------------|
| 229,616 | Switzerland | Feb. 1, 1944 |
|---------|-------------|--------------|